

Feb. 27, 1940.

J. R. JONES

2,191,962

PROCESS OF USING GRINDING GLASS SANDS

Filed March 28, 1938

*Fig. 1.*



*Fig. 2.*



Inventor  
JAMES R. JONES

By *Dorsey Cole & Garner*  
Attorneys

## UNITED STATES PATENT OFFICE

2,191,962

## PROCESS OF USING GRINDING GLASS SANDS

James Rudolph Jones, Kingsport, Tenn., assignor  
to Blue Ridge Glass Corporation, Kingsport,  
Tenn., a corporation of New York

Application March 28, 1938, Serial No. 198,589

2 Claims. (Cl. 51—278)

In the grinding and polishing of glass to form plate glass, sand (or similar substances) is frequently used as an abrading or polishing material, the sand being fed by water to the surface of the sheet of glass and rubber thereon by iron rubbers. In this operation the sand particles become broken and reduced in size. It has been the practice to pass the sludge coming from the grinding tables to sand graders with the purpose 5 of separating the sand particles according to their fineness, and the recovered products are again returned to the tables to be again used in grinding or polishing in accordance with their fineness. However, it has been noted that products 10 so recovered from the sludge do not possess the grinding and abrading power equal to fresh sand of the same particle size and this has been ascribed to the rounding of the sand particles in the preceding grinding and abrading operations.

I have discovered, however, that the inferiority 15 of the recovered sands is not due to this reason, but is due to the fact that the sand coming from a grinding table contains small particles of iron removed from the grinding heads in the grinding 20 of the glass. The classification or grading of the sand has been generally effected by subjecting a mixture of different grain size to the action of flowing water, the grading action being obtained 25 by selecting the velocity of the water in several settling tanks. Such a process of size grading is effective only if the particles treated are of uniform specific gravity. The iron particles due to 30 their high specific gravity are deposited in the several tanks along with said particles of much greater size.

My invention therefore contemplates the removal of the iron particles from the slurry coming from the grinding machines prior to the 35 grading of the grains thereof.

In the accompanying drawing in which corresponding marks of reference are used to indicate corresponding parts, Figure 1 is a diagrammatic representation of an apparatus suitable for carrying out this invention and

Figure 2 is a view of suitable magnetic separator.

A is a grinding table movable in the direction of the arrow on which is laid in the well known manner a layer of glass to be ground or polished. The movement of this table carries such glass beneath the rotating iron grinding heads C<sup>1</sup>, C<sup>2</sup> 5 and C<sup>3</sup> which are fed by a mixture of sand and water from the grading tanks D<sup>1</sup>, D<sup>2</sup> and D<sup>3</sup>. A suitable trough D is located beneath the grinding table for collecting the slurry resulting from the grinding operations of the several heads and this slurry is according to present practice returned to the first of the grading tanks D<sup>1</sup> by 10 means of the pump F and pipe line G. It is not thought necessary to describe the construction of the grading tanks as these may be of any 15 approved construction.

To avoid the deleterious effect which has been stated to result from the presence of iron particles in the sand there is located somewhere in this line, preferably at the sump H, a magnetic 20 separator I, a conventional showing of which is found in Figure 2 and which comprises a magnetized pulley i, the lower edge of which is immersed in the sludge and on the upper surface 25 of which bears a rubber scraper i<sup>b</sup>. The pulley attracts to it in its rotation the iron particles contained in the slurry and these are removed from the pulley by the scraper aided by water spray i<sup>b</sup> if desired.

Having thus described my invention what I 30 desire to secure by Letters Patent is:

1. The process of using glass grinding sands which involves feeding such sands to grinding heads in the presence of water, separating the iron particles contained in the slurry from the 35 grinding tables from the sand contained therein, classifying the sand according to its particle size and returning the graded sand to grinding heads in accordance with its grain size.

2. The hereinbefore described process which 40 comprises removing iron particles from the slurry of glass grinding machines, separating the sand remaining in the slurry according to particle size and feeding the separated sand to glass grinding heads.

JAMES RUDOLPH JONES.